

June 30, 1931.

W. B. BRAGGER ET AL

1,812,134

ORNAMENTAL MATERIAL, INSERT FOR SAME, AND METHOD OF MAKING SAME

Filed Jan. 10, 1930

Fig. 1.



Fig. 2.



Fig. 3.



Fig. 6.



Fig. 4.



Fig. 7.



Fig. 5.



Inventors

and  
William B. Bragger  
Victor F. Nekarda

James R. Bowen  
Attorney

## UNITED STATES PATENT OFFICE

WILLIAM B. BRAGGER, OF EXETER, MAINE, AND VICTOR F. NEKARDA, OF JERSEY CITY, NEW JERSEY, ASSIGNEES TO PEARL ART, INC., OF NEW YORK, N. Y., A CORPORATION OF NEW YORK

## ORNAMENTAL MATERIAL, INSERT FOR SAME, AND METHOD OF MAKING SAME

Application filed January 10, 1930. Serial No. 419,995.

The present invention relates to improvements in ornamental materials, inserts therefor, and methods of making same.

One object of the invention is to provide a material of ornamental character in which various colored and figurative effects may be obtained.

Another object of the invention is to provide an improved method of combining a mass and the inserts therein whereby a varied color effect may be had.

With the foregoing and other objects in view the invention will be more fully described hereinafter and will be more particularly pointed out in the claims appended hereto.

In the accompanying drawings,

Fig. 1 is a diagrammatic enlarged view of a part of a shell illustrating the laminations thereof;

Fig. 2 is a similar view showing a piece of shell cut across the laminæ thereof and exposing edges of such laminæ;

Fig. 3 is a top view illustrating serrated edges of overlapping laminæ of a shell piece;

Fig. 4 is a side view of a piece of shell after such piece of shell has been subjected to the action of coloring matter;

Fig. 5 shows an artificially colored shell piece imbedded into a mass at an angle to a break or cut across the laminæ of such shell piece, such shell piece being also shown as imbedded into a mass at an angle of a facet of the shell piece to a surface of the mass;

Fig. 6 illustrates shell pieces imbedded into a mass, laminæ of the shell pieces being shown at the same angle; and

Fig. 7 illustrates shell pieces imbedded into a mass, the laminæ of the shell pieces being shown at different angles.

In carrying our invention into effect inserts are placed in any suitable plastic mass susceptible of becoming set or hardened. Such plastic mass may consist of a single kind of material or may consist of a mixture of materials. As illustrative of plastic masses which may be used in carrying our invention into effect plastic masses of or containing casein, bakelite, metal alloy, cement, celluloid or clays may be mentioned. The plas-

tic mass may be given any desired color or colors, and the plastic mass may be such as will be susceptible to a polish after the plastic mass has set or hardened. The hardened mass will constitute a base of our ornamental material.

The inserts placed in the plastic mass are preferably pieces of shell of a translucent nature formed of laminæ having irregular surfaces which overlap one another, the edges of the laminæ of the pieces of shell being serrated and being disposed in zigzag formation as shown in Fig. 3. The irregular surfaces of the laminæ and the serrated edges of the laminæ may not be readily discerned with the naked eye but they may be apparent if subjected to microscopical examination. Through the phenomenon of light interference the irregularities in the surfaces of the laminæ and the zigzag formation of the edges of the laminæ cause light rays to split into their colored constituents and produce a characteristic chromatic iridescent nacreous effect.

In Fig. 1 15 designates the laminæ of a portion of a shell, and the arrows A indicate serrated edges of the laminæ of a portion of a shell. When the faces of the laminæ 15 and the serrated edges indicated by the arrows A are presented to rays of light to their broadest possible extent the chromatic iridescent nacreous effect above referred to will result; but if the laminæ 15 be cut, broken or ground at right angles to their layer formation as illustrated by the arrows B in Fig. 1 and only the cut, broken or ground edges of the layers of the laminæ be exposed to the light the chromatic iridescent nacreous effect above referred to will be at a minimum, resulting in a characteristic translucent milky lustre. And if the laminæ be cut, broken or ground at an angle within a ninety degree arc to the layer formation of the laminæ then, as the angle lessens from a right angle to the layer formation a larger and larger part of the faces and of the serrated edges of the laminæ will be exposed to the light and the translucent milky lustre will decrease, the chromatic iridescent nacreous effect increasing as the angle to the layer formation of the laminæ grows less. Fig. 2 is intended to repre-

55

60

65

70

75

80

85

90

95

100

sent a case where the line of the cut 16 across the laminæ is at an angle of say forty-five degrees to the layer formation of the laminæ of a piece of shell.

5 What we mean by the angle of the laminæ is the angle which the line of the break or cut across the laminæ (such line forming a facet) bears to the layer formation of the laminæ of the piece of shell.

10 The inserts may be imbedded in the plastic mass haphazardly and chances taken as to the angles, if any, which the outermost facet of each shell piece will bear to the layer formation of such shell piece when the shell piece is presented to view in the finished material. Or the inserts may be sorted and the basis for such sorting may be the angle which the facet of a piece of shell bears to the layer formation of such piece of shell, and pieces 15 of shell may be inserted in the plastic mass with a selected outermost facet of each piece of shell at a predetermined angle to the layer formation of such piece of shell. Obviously 20 an angle selected may be any within ninety degrees or there may be no angle at all if a facet chosen has the laminæ of its piece of shell as such laminæ are on the surface of such piece of shell.

25 The inserts may be so placed in the mass that when the material is in finished condition the laminæ presented to view in each selected outermost facet of each piece of shell will be presented at a predetermined angle to such selected outermost facet. And a 30 piece of shell may be placed in the mass not only with regard to the angle which a selected outermost facet bears to the layer formation of the laminæ of such piece of shell, but a shell piece may be so placed in the mass 35 that a selected outermost facet of such shell piece will be parallel or at any predetermined angle to a finished surface of the material.

40 Inserts may be so placed in the mass that the angle of the laminæ of each shell piece 45 will be uniform and of the same degree in each piece, or the shell pieces may be so placed in the mass that their respective laminæ will be at all angles or at varied desired angles within an arc of ninety degrees, resulting in the presentation to view on a finished surface of the material of a chromatic 50 kaleidoscopic effect ranging from a purely nacreous to a milky translucent effect.

55 In Fig. 6 pieces of shell are shown as placed in a plastic mass, the shell pieces illustrated in that figure being arbitrarily shown all at the same angle. In Fig. 7 three pieces of shell 60 17, 18 and 19, of arbitrary size and shape, are shown as placed in a mass 13. 17 is intended to represent a piece of shell placed in the mass with the laminæ presented by the selected outermost facet of such piece of shell in parallel relation to the line of such facet; 65 18 is intended to represent a piece of shell placed in the mass with the laminæ presented

by a selected outermost facet of such last mentioned piece of shell at an angle of say forty-five degrees to the line of such facet; and 19 is intended to represent a piece of shell 70 placed in the mass with the laminæ presented by a selected outermost facet of such last mentioned piece of shell at say an angle of ninety degrees to the line of such facet.

75 Shell pieces intended for use may be artificially colored. Coloring matter will not penetrate in a direction at right angles to the laminæ of the layer formation of a piece of shell except to an inappreciable extent if at all. Coloring matter will, however, penetrate to a greater or less extent in between the 80 laminæ of a piece of shell. The penetrability of coloring matter between laminæ, however, grows less and less from the edges of the laminæ. And while coloring matter will 85 penetrate inappreciably or not at all in a direction at right angles to the laminæ of a shell piece, the material of the shell piece is translucent and some trace of color will be 90 visible even in a facet of a shell piece which presents the laminæ of such shell piece parallel to the layer formation of such shell piece. Figs. 4 and 5 are intended to arbitrarily 95 show pieces of shell and to illustrate the decreasing penetration of coloring 22 between the laminæ 15 from the edges.

100 Artificially colored shell pieces may be placed in a plastic mass in the manner already described, but if artificially colored shell pieces are to be placed in a plastic mass in accordance with a predetermined plan there may be considered, in working out the results of such predetermined plan, not only the angles of the laminæ, as before explained, but the angle to the horizontal of a selected outermost facet. In Fig. 5 a piece of shell artificially colored, say green, is shown as placed in a mass with the laminæ of such piece of shell at a predetermined angle and with a selected outermost facet at a predetermined angle to the horizontal. I—E is a selected facet of 105 the shell piece illustrated and the angle which such selected facet bears to the horizontal.

110 Shell pieces intended for use may be of one or more varieties and of any desired color or shade of color, or any desired combination of colors or shades of color, and shell pieces of different varieties and of various colors or shades of color may be placed in the same mass. Artificially colored shell pieces and shell pieces not artificially colored may be placed in the same mass. Shell pieces may be placed in the mass in accordance with any predetermined design or pattern.

115 The pieces of shell used will be of adequate size to secure a good grip in the material.

120 The shell pieces may be placed in the mass manually or otherwise. Selected facets may, if desired, be lightly attached at predetermined angles to a matrix and that matrix

may thereafter be used in placing the pieces of shell in the mass.

Shell pieces may be so placed in the mass that parts of the shell pieces will protrude from the mass after it has hardened, but where shell pieces are so placed in the mass the shell pieces will penetrate sufficiently deep into the material so that no piece of shell may accidentally be pulled out. Or the shell pieces may be so placed in the plastic mass that the plastic mass will cover them.

After the shell pieces are placed in the plastic mass such mass will be permitted to harden.

After the mass has hardened such pieces of shell as protrude from the hardened mass may be reduced to the surface from which they protrude. The reduction of such protruding shell pieces may be accomplished by grinding or rubbing down the protruding shell pieces, and after the shell pieces have been reduced to the surface from which they protrude such shell pieces may be polished.

The hardened mass may be of any desired shape or form, and will, when finished, present to view one or more surfaces showing inserts therein.

Should pieces of shell have been so imbedded in the plastic mass as to be covered by such plastic mass, any desired surface of the mass, when hardened, may be reduced, as by grinding, rubbing or otherwise, to bring into view pieces of shell imbedded in such mass, and, as illustrated in Fig. 6, a surface of the hardened mass may be so reduced that the laminae of imbedded shell pieces may be ground across in a convex manner 20, in a concave manner 21, or at any angle.

Should artificially colored shell pieces have been imbedded in the mass, the reduction of a surface of the mass and with it the reduction of such artificially colored shell pieces as are affected by the reduction of such surface may result in the presentation to view of shell pieces of progressive degrees of vividness of color. For instance, if the laminae of the piece of shell illustrated in Fig. 4 be cut or ground down along the line C—D color as vivid, or substantially as vivid, as the coloring matter used will appear at point C and at point D the vividness of the color will be materially less. And if the mass into which the piece of shell illustrated in Fig. 5 has been imbedded be reduced from the surface indicated by the line G—H to the line indicated by the line J—K the imbedded piece of shell will have been reduced to the line F—E. The point E will have been slightly, if at all, affected in the reducing process but all the shell piece between the points I and F will have been ground or rubbed away before the point F is reached. The result will be that when a surface of the hardened mass is reduced to the line J—K the shell piece at point E will, for reasons

already explained, show a color substantially as vivid as the coloring used and this color will shade off along the line J—K from E to F, and at point F the color will be less vivid than at any point between E and F due to the fact that at point F the shell piece has been reduced to a point where the coloring 22 has penetrated between the laminae 15 of the shell piece to a lesser extent than anywhere else along the line from E to F.

The portions of pieces of shell exposed to view in the reduction of the hardened mass may be polished in the process which brings them into view, or the portions of the pieces of shell exposed to view may be polished after the reducing process.

If the hardened mass is susceptible to polish it and the portions of the pieces of shell exposed to view may be polished in the reducing process, or the hardened mass and the portions of the pieces of shell exposed to view may be polished after the reducing process has been completed.

Any suitable apparatus may be used in reducing a hardened mass or for giving a desired form or shape to the finished material, and if it be desired to polish pieces of shell presented to view or the surface of the hardened mass any suitable apparatus may be employed for either or both purposes.

After the treatment of the hardened mass has been completed it may, if desired, be coated with transparent material as, for instance, a transparent enamel.

The shell pieces become parts of the mass in which they are placed, and when the hardened mass has been reduced the parts of the shell pieces presented to view are integral parts of the surface or surfaces of the hardened mass exposed to view.

The ornamental material produced by our invention may be of any shape or form.

It is obvious that various changes and modifications may be made in the details of the above specifically described embodiment of the invention without departing from the spirit thereof.

We claim:

1. An ornamental material comprising a base and laminated structures imbedded in the base, an exposed facet of a laminated structure imbedded in the base being at an angle to the layer formation of the laminated structure having such exposed facet.

2. An ornamental material comprising a base and laminated structures imbedded in the base, exposed facets of laminated structures imbedded in the base being at an angle to the layer formation of the laminated structures having such exposed facets.

3. An ornamental material comprising a base and laminated structures imbedded in the base, laminae of a laminated structure imbedded in the base having coloring matter between such laminae.

4. An ornamental material comprising a base and laminated structures imbedded in the base, laminae of laminated structures imbedded in the base having coloring matter between such laminae.
5. An ornamental material comprising a base and laminated structures imbedded in the base, laminae of a laminated structure imbedded in the base having coloring matter between them and the coloring produced by such coloring matter varying in degree.
6. An ornamental material comprising a base and laminated structures imbedded in the base, laminae of laminated structures imbedded in the base having coloring matter between them and the coloring produced by such coloring matter varying in degree.
7. An ornamental material comprising a base and laminated structures imbedded in the base, laminae of a laminated structure imbedded in the base having coloring matter between such laminae and such laminae being at an angle to an exposed facet of such laminated structure.
8. An ornamental material comprising a base and laminated structures imbedded in the base, laminae of laminated structures imbedded in the base having coloring matter between such laminae and such laminae being at angles to exposed facets of such laminated structures.
9. The herein described method of making an ornamental material which consists in the introduction of coloring material between laminae of laminated structures, inserting such laminated structures in a plastic mass susceptible to hardening, permitting such mass to harden, and reducing a surface of the hardened mass.
10. The herein described method of making an ornamental material which consists in placing laminated structures in a plastic mass susceptible of hardening, imbedding a laminated structure in the mass with a facet thereof exposed and at an angle to the layer formation of the laminated structure having such exposed facet.
11. The herein described method of making an ornamental material which consists in placing laminated structures in a plastic mass susceptible of hardening, imbedding other laminated structures in the mass with facets thereof exposed and at an angle to the layer formation of the laminated structures having such exposed facets.

In testimony whereof we affix our signatures.

WILLIAM B. BRAGGER.  
VICTOR F. NEKARDA.